

Nov. 23, 1965

F. A. MARTIN

3,218,741

COATING FOR STEAM IRON FLASH BOILER

Filed Sept. 3, 1963



Fig. 1



Fig. 2



Fig. 3

## 1

3,218,741

COATING FOR STEAM IRON FLASH BOILER  
Frank A. Martin, Akron, Ohio, assignor to The Hoover  
Company, North Canton, Ohio, a corporation of Ohio  
Filed Sept. 3, 1963, Ser. No. 305,973  
7 Claims. (Cl. 38—77)

The present invention relates to coatings for the flash boiler of steam irons and to the method of applying such coatings.

In steam irons of the flash boiler type the water is fed drop by drop onto a hot spot on the sole plate, usually depressed below the top surface of the sole plate, and which constitutes the flash boiler.

If no means is provided to prevent it, the drops of water will roll about over the surface without being evaporated, and be ejected or spit onto the material being ironed in the form of water droplets which stains the material.

In the past the flash boiler has been coated with a hydrophilic material such as sodium silicate which prevents the spitting but eventually wears away.

According to the present invention the flash boiler is coated with mica flakes partially embedded in the metal of the sole plate and held in place to some extent by a binder.

The coating is applied to the die before the sole plate is cast and transferred to the sole plate during the casting operation thus doing away with a separate cooling operation after the sole plate is formed, which operation is expensive and time consuming.

According to the present invention a water suspension of a mixture of the mica and binder is sprayed onto the hot die (which is maintained at about 600° F.), at that point on the die which forms the flash boiler, the die closes and the castings immediately form.

The water forming the suspension is immediately evaporated, and the mica and binder deposited on the die as a coating. As the casting is formed, the coating is transferred to the casting and the mica partially embedded in the metal of the casting.

The primary purpose of the binder is to form the water suspension for the mica. The binder used is a white fluffy powder consisting mainly of colloidal alumina ( $Al_2O_3$ ) sold under the trade name of "Baymal."

Other objects and advantages of the present invention will become apparent as the description proceeds when taken in connection with the accompanying drawing in which:

FIG. 1 is a perspective view showing the die being coated.

FIG. 2 is a perspective view of the top of a sole plate; and

FIG. 3 is an enlarged cross-sectional view of the bottom of the flash boiler taken on line 3—3 of FIG. 2.

The female die 10 has a depressed portion 11 which forms the body 12 of the sole plate, a raised portion 13 which forms the flash boiler 14 connected to a raised portion 15 which forms the steam passages 16. A sprayer 17 of any suitable type is shown in FIG. 1 applying the suspension to an area limited to the raised portion 13 which forms the flash boiler 14, the coating being shown at 18.

The coating 19 of FIG. 3 was drawn from a micro-photograph of a section of the metal of the sole plate,

## 2

the section being cut through the bottom of the flash boiler.

As shown the tail ends of the mica flakes 20 are embedded in the metal of the sole plate and lie in overlapping or shingle like formation.

While in FIG. 3 the mica flakes 20 are shown in a regular arrangement the micro-photograph shows them in more of a haphazard arrangement but the general arrangement is clear.

10 A silica layer 21 overlies the flakes 20 with the flakes projecting above the surface of the silica as shown.

The "Baymal" and mica crystals are placed in a container, water added and the container agitated to form a suspension.

15 The sprayer 17 is of the air jet type of known construction. The liquid suspension is led to the sprayer 17 by tube 22 and air by tube 23.

The die 10 is maintained at about 600° F. and as the spray is applied the water is immediately evaporated leaving the coating 18 of mica and alumina mostly positioned on top of the raised portion 13 of the die. Of course the coating is not limited to that area but that is the area which it is desired to coat.

20 The die is immediately closed and the sole plate 12 cast. The coating 18 is transferred to the bottom 14 in the form of coating 19 in which the flakes 20 are arranged in shingle or fish scale like formation with their tail ends embedded in the metal of the sole plate and with their upper ends projecting above the layer 21 of alumina to form a roughened surface.

25 While I have shown and described but a single embodiment of my invention it is to be understood that that embodiment is to be taken as illustrative only and not in a limiting sense. I do not wish to be limited to the specific structure and method shown and described but wish to include all equivalent variations thereof except as limited by the scope of the claims.

I claim:

30 1. A sole plate for a steam iron, a flash boiler formed on said sole plate and a coating embedded in the surface of said flash boiler including mica flakes and an alumina binder for said mica flakes.

40 2. A sole plate for a steam iron, a flash boiler formed on the upper side of said sole plate and a coating on the surface of said flash boiler including mica flakes and alumina, said mica flakes being arranged in overlapping relationship with the tails thereof embedded in the metal of said sole plate and the upper ends exposed through said alumina.

45 3. The method of coating an aluminum casting comprising, maintaining a forming die at an elevated temperature, spraying said die with a coating material prepared in a water suspension whereby said water is evaporated and said coating material is deposited on said die, closing said die and immediately forming said casting whereby said coating material is transferred from said die to said casting.

50 4. The method according to claim 3 in which said coating material is a mixture of mica flakes and alumina.

55 5. The method of coating the flash boiler of a steam iron comprising, maintaining a casting die at an elevated temperature, forming a water suspension of a mixture of mica flakes and alumina, spraying that portion of said die which forms the flash boiler with said suspension whereby the water is evaporated and the mixture of mica

crystals and alumina is deposited on said die as a coating and casting said sole plate with said coated die whereby said coating is transferred to said casting as a coating for the flash boiler of said sole plate.

6. The method according to claim 5 in which said flakes are deposited in overlapping relation with the tail ends thereof embedded in the metal of said sole plate. 5

7. The method according to claim 6 in which said alumina forms a coating over said mica flakes with the upper edges of said flakes projecting above said coating. 10

## References Cited by the Examiner

## UNITED STATES PATENTS

|           |        |                 |       |         |
|-----------|--------|-----------------|-------|---------|
| 2,055,507 | 9/1936 | Shirley         | ----- | 117—160 |
| 2,075,388 | 3/1937 | De Cloud        | ----- | 117—160 |
| 2,568,004 | 9/1951 | Heyman          | ----- | 117—160 |
| 2,967,365 | 1/1961 | Extale et al.   | ----- | 38—77   |
| 3,101,561 | 8/1963 | Albrecht et al. | ----- | 38—77   |

JORDAN FRANKLIN, *Primary Examiner.*